# EUROPEAN PATENT SPECIFICATION

(11) **EP 2 889 060 B1**
(45) Date of publication and mention of the grant of the patent: **27.04.2016**
(21) Application number: 13199853.6
(22) Date of filing: 30.12.2013
(51) Int. Cl.: A63B 53/02, A63B 53/04, A63B 53/10

(54) **Method for assembling club head and shaft**
Verfahren zur Montage eines Golfschlägerkopfs und -schafts
Procédé d'assemblage de tête et manche de club

(43) Date of publication of application: 01.07.2015
(73) Proprietor: Hsu, Wen-Chien, 813 Kaohsiung City (TW)
(72) Inventor: Hsu, Wen-Chien, 813 Kaohsiung City (TW)
(74) Representative: Banse & Steglich

(56) References cited:
- GB-A- 2 267 221
- JP-A- H09 287 003
- JP-A- H10 146 404
- US-A- 5 665 014
- US-A1- 2010 181 368

## Description

### FIELD OF THE INVENTION

The present invention relates to a golf club, and more particularly to a method for assembling a club head and a shaft.

### BACKGROUND OF THE INVENTION

Recently, the sport of golf has become more and more popular in the world, especially for the young generation. The innovation of a golf club is flourishing as all manufacturers are trying their best to pursue a golf club able to hitting longer and swinging smoother.

A golf club is assembled by a club head and a shaft. A club head is primarily made of a metal an alloy, and a shaft is primarily classified as a carbon fiber shaft and a steel shaft in which there are generally three different hardness of a shaft can be found as a hardness of stiff flex (S), a regular/stiff flex (RS) and a regular flex (R). A stiffer shaft, which is less flexible, provides a more direct impact when a golf head is hitting a golf ball, so it can enhance a control of the ball, while it requires a faster swinging speed. On the contrary, a regular flex (R) shaft is easier to swing since it does not require a swinging speed so fast, but it is more difficult to obtain a long distance as compared with the stiff flex (S) shaft since a club shaft that is flexible will cause a varied swinging path to thus reduce a control of a golf club.

However, no matter what kinds of material a golf club is, the conventional golf club is assembled by means of sleeve-connecting for adhering a club head and a shaft. Such construction is unable to provide a mechanically perfect assembly due to different materials of the club head and the shaft, which may cause a sound of friction or even a crash in the connection therebetween while a hard swing. In addition that the joint area between the club head and the shaft has a high risk of separation or crash resulted from a stress concentration thereon, the way of jointing the club head and the club shaft may also result in a deviation of a ball path if there is only a small slit existed there between.

The documents GB2267221 and US2010/181368 disclose a golf club with the shaft connected to the club head, by means of press-fitting or adhesives.

### SUMMARY OF THE INVENTION

In view of the above, it is an object of the present invention to provide a method for assembling a club head and a shaft to improve the assembling effect thereof.

Therefore, the present invention overcomes the technical problems in the conventional art and provides a method for assembling a club head and a shaft, comprising: a step of jointing a blank element of club head with a blank element of shaft that are made of different materials to construct a blank element of golf club; a step of wrapping up the blank element of golf club with powder by used of a wrapping member; and a step of constructing a golf club by applying an isostatic pressing to the wrapped up blank element of golf club to construct the blank element of club head, the blank element of shaft and the powder as a golf club.

According to an embodiment of the present invention, the blank element of club head and the blank element of shaft are made of metals with different materials, alloys with different compositions, alloys with the same composition but with different ratios thereof, or metals/alloys made by different processes.

According to an embodiment of the present invention, in the jointing step, the blank element of club head and the blank element of shaft are jointed by attaching their radial surfaces with each other or fastening with fastening portions with each other.

According to an embodiment of the present invention, the wrapping step is processed by pre-forming the powder as an wrapped blank element, or by a vibration that fills the powder into the wrapping member.

According to an embodiment of the present invention, the powder is a metallic powder.

According to an embodiment of the present invention, the wrapping step further includes a sub-step of sealing that seals the wrapping member.

According to an embodiment of the present invention, the wrapping member is made of a metallic material or a ceramic material.

According to an embodiment of the present invention, the isostatic pressing is a hot isostatic pressing with a high temperature and a high pressure.

With the characteristic features as above, the present invention provides a golf club in which a club head and a shaft made of different materials can be assembled as a strong and hard connected golf club with respect to a mechanical effect to thus reduce a stress concentration and reduce a risk of crash in the joint portion. In addition, a force transmission of the present invention can be smoother so that a precision degree of control with respect to a golf club can be improved.

### BRIEF DESCRIPTION OF THE DRAWINGS

The structure and the technical means adopted by the present invention to achieve the above and other objects can be best understood by referring to the following detailed description of the preferred embodiments and the accompanied drawings.
Fig. 1 is a flow chart illustrating a method for assembling a club head and a shaft according to one embodiment of the present invention.
Figs. 2a to 2c are schematic diagrams illustrating a jointing step of the method according to the embodiment of the present invention;
Fig. 3 is a schematic diagram illustrating a wrapping step of the method according to the embodiment of the present invention;
Fig. 4 is a schematic diagram illustrating a constructing step of the method according to the embodiment of the present invention; and
Fig. 5 is a schematic diagram illustrating a golf club constructed by the method according to the embodiment of the present invention.

### DETAILED DESCRIPTION OF THE PREFERRED EMBODIMENTS

Embodiments are described in detail as below in reference to Figs. 1 to 5, and the description is used for explaining the embodiments of the present invention only but not for limiting the scope of the present invention.

As shown in Fig. 1, a method for assembling a club head and a shaft according to one embodiment of the present invention comprises: a jointing step S10, a wrapping step S20 and a constructing step S30. The method of the present invention is mainly used for assembling a club head and a shaft made of different materials that are assembled stably and firmly with a mechanical property of a smooth force transmission.

Next, the method will be described below in accordance with an embodiment of the present invention with reference to Figs. 2a to 5.

First, as shown in Figs. 2a to 2c, the jointing step S10 is processed to joint a blank element of club head 1 and a blank element of shaft 2 both of which are made of different materials to thereafter construct a blank element of golf club, wherein the different materials are referred to materials having different properties. For example, in the embodiment, the blank element of club head 1 and the blank element of shaft 2 are made of metals that are with different materials, alloys that are with different compositions, alloys that are with the same composition but are with different ratios thereof, or metals/alloys made by different processes including casting, forging, or drawing, etc..

The blank element of club head 1 and the blank element of shaft 2 may be jointed by attaching a radial surface of a connecting hole of the blank element of club head 1 with a radial surface of the blank element of shaft 2, or alternatively by fastening with fastening portions of the blank element of club head 1 and the blank element of shaft 2. As shown in Fig.2a, during the attaching process, a blank element of club head 1 has a connecting portion 11, a blank element of shaft 2 has a receiving portion 21, and the connecting portion 11 is connected to the receiving portion 21. A jointing depth between the blank element of club head 1 and the blank element of shaft 2 is adjustable with respect to the material properties thereof. As shown in Fig. 2b, a jointing depth between a connecting portion 11a of a blank element of club head 1 and a receiving portion 21a of a blank element of shaft 2 may be substantially equal to a length of the blank element of shaft 2. As shown in Fig. 2c, during the fastening process, a blank element of club head 1 is with a fastening portion 12, a blank element of shaft 2 is with a fastened portion 22, and the fastening portion 12 is fastened to the fastened portion 22 to joint the blank element of club head 1 with the blank element of shaft 2. However, the present invention is not intended to limit these. A blank element of club head 1 and a blank element of shaft 2 can be alternatively jointed by other conventional jointing manners or a novel jointing manner.

After the jointing step S10, the wrapping step S20 will be processed. In the embodiment, the wrapping step S20 primarily includes: a wrapping sub-step S21 and a filling sub-step S22.

In the wrapping sub-step S21, a wrapping member 3 is used to wrap the blank element of golf club that is constructed by the blank element of club head 1 and the blank element of shaft 2. The wrapping member 3 may be made of a ceramic material or a metallic material including: a mild steel, a stainless steel, Titanium, etc. A metallic wrapping member is suitable for constructing a golf club with simple shape, and a ceramic wrapping member is suitable for a golf club with a sophisticated or a complicated shape.

As shown in Fig. 3, the filling sub-step S22 is processed to fill the powder 40 into the wrapping member 3 in order to wrap the blank element of golf club. Optionally, the material of powder 40 can be varied depending on the blank element of club head 1 and the blank element of shaft 2, such as metal or ceramic. In this embodiment, the powder 40 is a metallic powder. There are mainly two ways for filling the powder. One is for pre-forming the powder 40 as a wrapped blank element (not shown), and thereafter the blank element of golf club is wrapped in the wrapped blank element, and accordingly the wrapped blank element is wrapped in the wrapping member 3. The other way is to fill the powder 40 into an interval space between the wrapping member 3 and the blank element of golf club by means of a vibration, and fill in a gap between the blank element of club head 1 and the blank element of shaft 2 as well.

Preferably, after the filling step S22, a sealing sub-step S23 may be processed. The sealing sub-step S23 is for sealing the wrapping member 3. Sealing is usually processed by means of seal welding. Before processing the sealing step, it requires to vacuum evacuate the wrapping member 3 in a room temperature or in a heating environment to construct a close direct contact among the wrapping member 3, the blank element of golf club and the powder 40 to prevent cavities generated thereamong to improve the quality of a golf club.

Next, after the wrapping step S20, the constructing step S30 will be processed. The constructing step S30 is to apply an isostatic pressing to the wrapped blank element of golf club to construct an integral structure with the blank element of club head 1, the blank element of shaft 2 and the powder 40. The isostatic pressing referred herein is a hot isostatic pressing with a high temperature and a high pressure. As shown in Fig. 4, an wrapped blank element of golf club is placed into a processing vessel 5 in which a gas is then introduced and is followed by a heating process, in which the powder 40 and the wrapped blank element of golf club is isostatically pressed by a high pressure generated by a thermal expansion of the gas. By means of the isostatic pressing, the powder 40 wrapping up the blank element of golf club will be sintered as a densely sintered body 4 that is densely covering the blank element of club head 1 and the blank element of shaft 2.

Finally, as shown in Fig. 5, after the constructing step S30, an ejecting step S40 will be processed to eject the densely sintered body 4 and the blank element of golf club from the wrapping member 3 to thus obtain a golf club 100 in which a club head and a shaft made of different materials are assembled.

In the golf club 100, gaps and cavities between a golf club head and a golf shaft have been eliminated, and an exterior surface at a jointing portion between the golf club head and the golf shaft became an integrated smooth surface. The golf club 100 has mechanical assembling property similar to a single-piece golf club in which it reduces a stress concentration and a risk of crash in the joint portion, and therefore a force can be transmitted smoother so that a precision degree of control with respect to the golf club can be improved.

The above description should be considered as only the discussion of the preferred embodiments of the present invention. However, a person with an ordinary skill in the art may make various modifications to the present invention, but such modifications should be considered as falling within the scope defined by the appended claims.

## Claims

1. A method for assembling a club head and a shaft, comprising:
a step of jointing a blank element of club head with a blank element of shaft that are made of different materials to construct a blank element of golf club;
a step of wrapping up the blank element of golf club with powder by used of a wrapping member; and
a step of constructing a golf club by applying an isostatic pressing to the wrapped up blank element of golf club to construct the blank element of club head, the blank element of shaft and the powder as a golf club.

2. The method as claimed in claim 1, wherein the blank element of club head and the blank element of shaft are made of metals with different materials, alloys with different compositions, alloys with the same composition but with different ratios thereof, or metals/alloys made by different processes.

3. The method as claimed in claim 1, wherein in the jointing step, the blank element of club head and the blank element of shaft are jointed by attaching their radial surfaces with each other or fastening with fastening portions with each other.

4. The method as claimed in claim 1, wherein the wrapping step is processed by pre-forming the powder as an wrapped blank element, or by a vibration that fills the powder into the wrapping member.

5. The method as claimed in claim 1, wherein the powder is a metallic powder.

6. The method as claimed in claim 1, wherein the wrapping step further includes a sub-step of sealing that seals the wrapping member.

7. The method as claimed in claim 1, wherein the wrapping member is made of a metallic material or a ceramic material.

8. The method as claimed in claim 1, wherein the isostatic pressing is a hot isostatic pressing with a high temperature and a high pressure.

## Patentansprüche

1. Verfahren zum Zusammenbau eines Schlägerkopfs und eines Schafts, umfassend:
einen Schritt zur Verbindung von einem Schlägerkopfrohling mit einem Schaftrohling, welche aus unterschiedlichen Materialien hergestellt sind, um ein Golfschlägerrohling zu konstruieren,
einen Schritt zum Umhüllen des Golfschlägerrohlings mit einem Pulver unter Verwendung eines Mantelelements und
einen Schritt zur Herstellung eines Golfschlägers durch Anwendung eines isostatischen Pressvorgangs auf den umhüllte Golfschlägerrohling, um aus dem Schlägerkopfrohling, dem Schaftrohling und dem Pulver einen Golfschläger herzustellen.

2. Verfahren nach Anspruch 1, bei welchem der Schlägerkopfrohling und der Schaftrohling aus verschiedenartigen Metallen, Legierungen mit unterschiedlichen Zusammensetzungen, Legierungen, welche die gleiche Zusammensetzung, aber unterschiedliche Verhältnisse aufweisen, oder aus Metallen/Legierungen, die durch verschiedene Verfahren gefertigt wurden, hergestellt sind.

3. Verfahren nach Anspruch 1, bei welchem der Schlägerkopfrohling und der Schaftrohling in dem Schritt zur Verbindung durch Befestigen ihrer Radialflächen aneinander oder durch Zusammenfügen mittels Befestigungsbereichen miteinander verbunden werden.

4. Verfahren nach Anspruch 1, bei welchem der Schritt zum Umhüllen ausgeführt wird, indem das Pulver als ein Mantelrohling vorgefertigt wird, oder indem eine Vibration erfolgt, durch welche das Pulver in das Mantelelement eingefüllt wird.

5. Verfahren nach Anspruch 1, bei welchem das Pulver ein metallisches Pulver ist.

6. Verfahren nach Anspruch 1, bei welchem der Schritt zum Umhüllen ferner einen Teilschritt zur Abdichtung beinhaltet, bei dem das Mantelelement abgedichtet wird.

7. Verfahren nach Anspruch 1, bei welchem das Mantelelement aus einem metallischen Material oder einem keramischen Material hergestellt ist.

8. Verfahren nach Anspruch 1, bei welchem der isostatische Pressvorgang ein heiß-isostatischer Pressvorgang bei einer hohen Temperatur und einem hohen Druck ist.

## Revendications

1. Procédé pour assembler une tête de club et un manche comprenant :
une étape d'assemblage d'une ébauche de tête de club à une ébauche de manche qui sont faits en différents matériaux pour construire une ébauche de club de golf ;
une étape d'emballage de l'ébauche de club de golf avec de la poudre en utilisant un élément d'emballage et
une étape de construction d'un club de golf en appliquant une compression isostatique à l'ébauche emballée de club de golf pour construire l'ébauche de tête de club, l'ébauche de manche et la poudre en tant que club de golf.

2. Procédé selon la revendication 1, l'ébauche de tête de club et l'ébauche de manche étant faites en métaux avec différents matériaux, en alliages de différentes compositions, en alliages de même composition mais avec différents rapports de ceux-ci, en métaux/alliages faits par différents processus.

3. Procédé selon la revendication 1, cependant que, dans l'étape d'assemblage l'ébauche de tête de club et l'ébauche de manche sont assemblées en attachant leurs surfaces radiales l'une à l'autre ou en les fixant avec des portions de fixation l'une à l'autre.

4. Procédé selon la revendication 1, cependant que l'étape d'emballage est effectuée en préformant la poudre en tant qu'ébauche emballée ou par une vibration qui remplit la poudre dans l'élément d'emballage.

5. Procédé selon la revendication 1, cependant que la poudre est une poudre métallique.

6. Procédé selon la revendication 1, cependant que l'étape d'emballage comprend de plus la sous-étape de scellement qui scelle l'élément d'emballage.

7. Procédé selon la revendication 1, cependant que l'élément d'emballage est fait en un matériau métallique ou en un matériau céramique.

8. Procédé selon la revendication 1, cependant que la compression isostatique est une compression isostatique à chaud avec une température élevée et une pression élevée.
